

Sept. 26, 1944,

K. S. KNOL ET AL

2,359,224

ELECTROMAGNETIC DEVICE

Filed April 12, 1941



INVENTORS  
KORNELIS S. KNOL  
MAXIMILLIAN J. O. STRUTT  
BY *H. S. Grover*  
ATTORNEY

## UNITED STATES PATENT OFFICE

2,359,224

## ELECTROMAGNETIC DEVICE

Kornelis Swier Knol and Maximiliaan Julius Otto  
Strutt, Eindhoven, Netherlands; vested in the  
Alien Property Custodian

Application April 12, 1941, Serial No. 388,250  
In the Netherlands April 29, 1940

2 Claims. (Cl. 176—45)

This invention relates to an electro-magnetic device such as a coil or a conductor and has for its purpose to raise the inductance of such a device at frequencies exceeding  $10^9$  cycles/sec. and more particularly by making use of ferromagnetic material.

According to the invention this purpose is attained by making use of layers of coherent ferro-magnetic particles applied on to a support.

When measuring the alternating current resistance of thin solid iron wires at high frequencies the magnetic permeability can be calculated from the resistance values obtained. Many investigators ascertained by means of such resistance measurements that the permeability at room temperature at frequencies of several cycles/sec. up to about  $10^8$  cycles/sec. is constant. Above  $10^8$  cycles/sec., however, the permeability exhibits a rapid drop of the initial value (for instance 100) to unity. Consequently it is unfeasible to utilise thin iron wires for raising the inductance, for instance of coils designed for frequencies above say  $10^9$  cycles/sec.

Researches made by us on layers consisting of coherent particles of ferro-magnetic material, which were applied on to a support by means of electrolysis, have proved that the permeability of such layers begins to drop at much higher frequencies than the permeability of thin iron wires, so that such layers may advantageously be used at frequencies above  $10^9$  cycles/sec.

It is of importance that the layers should be made in such manner that the ferro-magnetic particles of which they are formed stick together so that these layers have a metallic appearance. In a suitable method of manufacture a solution of 50 parts by weight of  $\text{FeCl}_2$ , 50 parts by weight of  $\text{CaCl}_2$  and 75 parts by weight of distilled water was made to boil and subsequently filtered. After that the electrolysis was effected at a temperature of the bath of about  $90^\circ \text{C}$ ., a cylindrically curved piece of iron plate of pure iron constituting the anode and a constantan wire, for instance, serving as a cathode. The current density amounted to about 30 ma./cm.<sup>2</sup> on the last-mentioned wire. The constantan wire to be coated was previously treated with a degreasing agent, pickled in diluted hydrochloric acid, washed in distilled water and immediately subjected to the electrolytic treatment. If this method is carried out carefully and as pure as possible solutions are used dense coherent iron layers are obtained which under a metal microscope (with a magnification of about 100) exhibit a metallic appearance which is only

slightly different from the surface of solid iron wires. By resistance measurements the specific resistance and its dependency with respect to temperature could be determined from the thickness of the layer also determined microscopically. In this way, also, perfectly coherent layers of pure iron are found. The thickness of the layer must exceed 1.5 microns.

Iron layers can be precipitated electrolytically also on iron wires, it being advisable that the iron wires to be coated should previously be coppered electrolytically.

In the drawing, Fig. 1 shows a coated wire or conductor in accordance with the invention, and Fig. 2 shows the relation between permeability and frequency for such a wire.

In Fig. 1, there is shown at 1 the wire of iron or constantan upon which there is deposited by the method above described a layer or a coating 2 of dense coherent particles of ferromagnetic material.

The curve 3 in Fig. 2 indicates the initial permeability  $\mu$  in accordance with the frequency  $f$  of an iron layer made in the manner referred to above. Therefrom it appears that the initial permeability up to  $10^9$  cycles/sec. is substantially constant and then gradually decreases, but at  $10^{10}$  cycles/sec. still has the very high value of about 80.

30 The wires coated with a layer of precipitated iron particles have an increased inductance and may, for instance, be used in amplifying tubes for short waves in which it is sometimes desirable to increase the inductance of the supply conductors for one or more electrodes of these tubes.

Furthermore layers precipitated on wires or plates may be formed into cores for coils used at frequencies above  $10^9$  cycles/sec.

40 It is to be noted that the layers may be made not only of iron, but also of other ferro-magnetic materials such as nickel, iron-nickel and so on.

Instead of applying the layers electrolytically they may also be provided on their supports by cathode disintegration or electrophoresis.

What we claim is:

1. An electrical conductor comprising a metallic support, a layer of dense coherent ferromagnetic particles on said support formed by electrolysis at current densities of approximately 30 ma./cm.<sup>2</sup>, said layer having a thickness in excess of 1.5 microns and a permeability of substantially 100 for a range of frequencies from zero up to approximately  $10^9$  cycles/second.

2. A high frequency conductor comprising a constantan wire provided with an outer coating of coherent particles of ferro-magnetic material formed by electrolysis at current densities of approximately 30 ma./cm.<sup>2</sup>, said coating having a thickness in excess of 1.5 microns, and said coating having a permeability of approximately 100

over a range of frequencies from zero up to approximately  $10^8$  cycles/second and which thereafter gradually decreases to about 80 to approximately  $10^{10}$  cycles/second.

**KORNELIS SWIER KNOL.  
MAXIMILIAAN JULIUS OTTO STRUTT.**